

## UNITED STATES PATENT OFFICE

2,212,178

ALLOY SUITABLE FOR USE AS BEARING  
METALS

Paul Kemp, Vienna, Germany

No Drawing. Application July 21, 1938, Serial  
No. 220,562. In Austria July 21, 1937

3 Claims. (Cl. 75—166)

This invention relates to alloys suitable for use as bearing metals.

The suitability of alloys as bearing metals is in general determined by investigation of a series of properties which have been recognised to be essential. Essential requirements are a sufficiently high resistance to compression to ensure the alloys withstanding the occasionally high surface pressures, a certain hardness, to ensure sufficient resistance being offered to the squeezing out of the metal from the bearing, and also sufficient upsetting and transverse strength which serves as a standard for the tenacity of the alloy, this last property being of very great importance, particularly in the case of strong impact stresses. In addition thereto, the sliding properties, capability of being satisfactorily cast and economic considerations play a corresponding part.

In view of the foregoing, the established fact that alloys, which with regard to all the above indicated properties fulfil the conditions required of satisfactory bearing metals and which also showed no appreciable differences from one another, behave quite differently in operation, was surprising. Above all it was observed that in bearings, which are exposed to impacts, some of these alloys developed cracks and in part also crumbled out, whilst others completely withstood the stresses.

According to this invention, it has been found that an adequately high bending strength together with a certain compressibility are not sufficient indications of the suitability of an alloy for bearings exposed to impacts. In actual fact also in the investigation of these two properties the procedures taking place in practical operation are only very incompletely represented, since, whilst the impacts and percussions occur suddenly in the bearing, the determination of the bending strength and compressibility requires a period of a few minutes.

The working conditions are much better represented in the percussion test. There are no standards for carrying out this test for bearing metals and, since it was only a question of comparative tests and not of the determination of absolute values, the applicant's investigations were therefore carried out with an arbitrarily selected drop hammer, in such a way that the latter was allowed to fall from the same height and at equal intervals of time onto a rod supported at two positions. The number of impacts required for breaking the rod was taken as the value of the resistance to percussion or percussion strength.

As a result of these investigations it was found that alloys, which showed only slight differences in bending strength and compressibility, occasionally varied very considerably in their percussion strength and that alloys having a high percussion strength are best adapted for bearings exposed to percussion or impacts.

Experiments carried out systematically showed that in order to obtain sufficient percussion strength in alloys of the three component system lead-antimony-tin, the antimony content together with that of the elements arsenic and cadmium advantageously admixed as hardening constituents, must not exceed the tin content and that the lead content must amount to at least 80%.

On the other hand it has in general been found to be advisable, in order to obtain as favourable hardness and strength as possible, that the quantity of antimony in the alloy together with the quantity of the arsenic and/or cadmium should not be substantially less than the quantity of tin present. A content of copper up to 2% has no influence on the percussion strength of these alloys. The composition of these alloys particularly adapted as bearing metals, must accordingly be maintained approximately within the following limits:

|                                    |                                                                                 |    |
|------------------------------------|---------------------------------------------------------------------------------|----|
| Lead                               | 80-86%                                                                          | 30 |
| Tin                                | 10-6% preferably 9-7%                                                           |    |
| Antimony plus arsenic plus cadmium | 10-6% preferably 9-7% of which Sb=7-6%, of which As=1-0.5%, of which Cd=1-0.7%. | 35 |

If desired, up to 2%, preferably only up to 1.5% of copper in addition.

By altering the proportions of the components in the above indicated limits, the hardness of the alloy can be extensively influenced. The lower the content of tin and accordingly also the contents of Sb, As and Cd, the lower is the hardness of the alloy. In the case of arsenic addition up to 1% and in the case of cadmium addition up to about 1.5% are suitable, but the sum of these two additional metals must not exceed 2%, since no particular advantages are obtained thereby.

Bearing metals of the same alloy system having a low content of copper have already been proposed, particularly in the applicant's Austrian Patents Nos. 130,903 and 135,895 and U. S. A. Patent No. 1,754,364. The alloys according to these patents, however, differ considerably from the alloys according to this invention in their

very much lower lead content, whilst on the other hand their content of antimony plus arsenic plus cadmium exceeds the upper limit according to this invention.

5 A comparison of the six-component system alloy (I) indicated in Austrian Patent No. 130,903 as optimum and having the composition: 10.4% of Sn, 9.8% of Sb, 1.45% of Cu, 1.5% of Cd, 1.2% of As and 75.65% of Pb, with an alloy 10 (II) according to the present invention, for example: 9% of Sn, 7% of Sb, 1.3% of Cu, 1% of Cd, 0.7% of As and 81% of Pb shows that the former under the same testing conditions breaks after three impacts whilst the latter only breaks 15 after 15 impacts.

With regard to the resistance to compression and bending strength, no appreciable differences exist between the two alloys, the latter alloy being merely somewhat softer. This lower hardness is however, not the cause of the higher 20 percussion strength, since for example alloy (III), 8% of Sn, 10% of Sb, 1.5% of Cu, 0% of Cd, 1% of As and 78.5% of Pb, which possesses the same hardness as the above alloy (II) likewise 25 breaks after only three impacts.

It must be assumed that the better properties of the alloys according to the present invention are occasioned inter alia by small quantities of free lead in the texture. In alloys having a lower 30 lead content, lead cannot occur as a constituent

of the texture, since it is entirely used up for the formation of the ternary Pb-Sb-Sn-Eutectic. Moreover, the known bearing metals of this system all contain a substantially higher quantity of antimony, which gives rise to the formation of more brittle crystals. The alloys according to the present invention are free from all the disadvantages of these known alloys. Moreover, owing to their higher lead content, they have the economic advantage of lower cost.

What I claim is:

1. A bearing alloy characterized by a high resistance to impact stresses consisting of 80% to 86% of lead, 10% to 6% of tin, up to 2% of copper and 10% to 6% of antimony and at least one of the metals cadmium and arsenic, the amount of arsenic being at most 1%, the amount of cadmium being at most 1.5%, and the quantity of arsenic and cadmium together being at most 2%.

2. A bearing alloy characterized by a high resistance to impact stresses consisting of about 7% to 9% of tin, 6% to 7% of antimony, 0.5% to 1.0% of arsenic, 0.7% to 1.0% of cadmium, up to 1.5% of copper and the remainder lead.

3. A bearing alloy characterized by a high resistance to impact stresses consisting of 81% of lead, 9% of tin, 7% of antimony, 0.7% of arsenic, 1% of cadmium and 1.3% of copper.

PAUL KEMP.